

March 21, 1933.

J. P. BROCKWAY

1,902,213

PROCESS OF REPRODUCING IMAGES ON METALLIC SURFACES

Filed Feb. 28, 1929

FIG. 1.



FIG. 2.



FIG. 3.

FIG. 4.



INVENTOR  
JOHN P. BROCKWAY  
BY  
*A. B. Bowman*  
ATTORNEY

## UNITED STATES PATENT OFFICE

JOHN P. BROCKWAY, OF CORONADO, CALIFORNIA, ASSIGNOR TO A. B. BOWMAN, OF SAN DIEGO, CALIFORNIA

## PROCESS OF REPRODUCING IMAGES ON METALLIC SURFACES

Application filed February 28, 1929. Serial No. 343,576.

My invention relates to a process of reproducing images on metallic surfaces, more particularly copper surfaces, and the objects of my invention are: First, to 5 provide a new and novel process of reproducing images; Second, to provide a new and novel process of reproducing images on metallic surfaces; Third, to provide a new and novel process of reproducing images on 10 metallic polished surfaces; Fourth, to provide a new and novel process of preparing film or negatives for reproducing from said film or negative on metallic surfaces; Fifth, to provide a new and novel process of fixing 15 the image on said metallic surface, and Sixth, to provide a new and novel process of this class which is very simple, efficient and economical of operation, effective, and which produces surfaces with images which are very 20 durable.

With these and other objects in view as will appear hereinafter, my invention consists of the certain novel process as will be hereinafter described in detail and particularly set forth in the appended claims, reference being had to the accompanying drawing which form a part of this application in which:

Figure 1 is a diagrammatic view of a chlorine gas supply container; Fig. 2 is a sectional view of a printing frame illustrating the facilities used in my process; Fig. 3 is a diagrammatic view of my electrical fixing bath apparatus; and Fig. 4 is an edge view of the 35 finished metal plate with the lacquer coating.

My process consists in taking an unsensitized photographic film of convenient size, a film 1 whose emulsion contains no salts of silver or other sensitizing chemical, and immersing said film in dry chlorine gas for an hour or more as shown in Fig. 1 of the drawing; then placing this film on any highly polished metallic surface, such as iron, steel, Monel metal, brass or copper, as designated 40 2 in Fig. 2 of the drawing preferably copper; then placing on this surface a negative 3 with a picture or images; these may be bound together in a photographic printing frame 4, or supported in their relation to each other 45 50 otherwise; and then exposing the same to

sunlight 5, or other similar light 5. The light will cause the adsorbed chlorine gas in the film 1 to become active and will print out the picture design or image contained in the negative on the metallic surface as shown in Fig. 55 3. After the picture or image has been printed out or made on the metallic surface it may be made permanent or fixed by electricity as follows:

The object 2 with the picture or image is 60 immersed in a bath of distilled water, 1500 cubic centimeters, nickel ammonium sulphate, 5 grams, sodium chromate, 5 grams, and ammonium bisulphate, 5 grams, which will form a bath. A plate forming an anode 65 is placed in the bath and said treated surface is used as a cathode and subjected to a current of electricity of 10 or more volts D. C. for a second or more of time, which will render the picture permanent, all as shown 70 in Fig. 3. The treated surface is immediately removed from the bath and thoroughly washed in running water and dried; then said surface is covered with a fine, transparent lacquer 6 as shown in Fig. 4 to prevent 75 marring or scraping of said surface.

In some cases, if desired, the film may be omitted and the negative may be subjected to or immersed in dry chlorine gas for an hour or more and the negative placed next to the 80 highly polished metal surface and exposed to the light, as hereinbefore described.

In the place of a photographic film treated in the manner above described, any other transparent sheet, capable of absorbing the 85 gas and remaining inert thereto, may be employed, as for example, celluloid, or transparent paper.

When desired to reproduce an enlarged 90 image from a negative the image is thrown onto the absorbent film placed over the metallic surface, by means of a conventional enlarging apparatus. The negative is of course not in contact with the gas treated film in this case.

Though I have described a particular process of reproducing images on metallic surfaces, I do not wish to be limited to this particular process, but desire to include in the scope of my invention the process substan- 95 100

tially as set forth in the appended claims.

Having thus described my invention, what I claim as new and desire to secure by Letters Patent is:

- 5 1. The herein described process of reproducing images on metallic surfaces, comprising the subjecting of a film to dry chlorine gas for a period of an hour or more, then placing the same on a highly polished metal-  
10 lic surface the metal of a group consisting of iron, steel, Monel metal, brass and copper, then placing a negative with images thereon over said chlorine treated film and subjecting the same to light.
- 15 2. The herein described process of reproducing images on metallic surfaces, comprising the subjecting of a film to dry chlorine gas for a period of an hour or more, then placing the same on a highly polished me-  
20 tallic surface the metal of a group consisting of iron, steel, Monel metal brass and copper, then placing a negative with images thereon over said chlorine treated film and subjecting the same to light, then placing said me-  
25 tallic surface in a bath compounded as fol-  
lows, distilled water, 1500 cubic centimeters, nickel ammonium sulphate, 5 grams, sodium chromate, 5 grams, and ammonium bisul-  
30 phate, 5 grams, and while submerged in said  
bath subjecting said surface to a current of  
electricity of 10 volts for one second, then  
washing the metallic surface and drying the  
same, then covering said surface with a fine,  
35 transparent lacquer.
- 35 3. The herein described process of repro-  
ducing images on metallic surfaces, comprising providing a metal of a group consisting of iron, steel, Monel metal, brass and copper with a highly polished surface, then subject-  
40 ing a transparent member to dry chlorine gas  
for a period of an hour or more, then placing  
said transparent member against said  
surface, then placing a negative with an  
image in contact with said chlorine gas  
45 treated film and then subjecting the same to  
light, then electroplating said surface.
4. The herein described process of repro-  
ducing images on metallic surfaces, comprising providing a metal of a group consisting  
50 of iron, steel, Monel metal, brass and copper with a highly polished surface, then subjecting a transparent member to dry chlorine  
gas for a period of an hour or more, then placing said transparent member against said  
55 surface, then placing a negative with an  
image in contact with said chlorine gas treat-  
ed film, then subjecting the same to light,  
then electroplating said surface, then cover-  
ing said surface with a transparent lacquer.
- 60 5. The herein described process of repro-  
ducing images on copper surfaces, comprising providing said copper with a highly  
polished surface, then placing a film with  
images on said surface and subjecting it to  
65 light and registering said image in light and

shadow on said surface in the presence of dry adsorbed chlorine gas for reproducing said image in tangible form on said surface.

6. The herein described process of repro-  
ducing images on copper surfaces, comprising providing said copper with a highly  
polished surface, then subjecting a film with  
images to light and registering said image in  
light and shadow on said surface in the pres-  
ence of dry adsorbed chlorine gas for re-  
producing said image in tangible form on  
70 said surface, then fixing said image on said  
surface by subjecting the same to an electric  
current while said surface is immersed in a  
bath compounded as follows, distilled water,  
75 1500 cubic centimeters, nickel ammonium  
sulphate, 5 grams, sodium chromate, 5 grams,  
and ammonium bisulphate, 5 grams.

7. The herein described process of repro-  
ducing images on copper surfaces, comprising providing said copper with a highly  
polished surface, then subjecting a film with  
images to light and registering said image in  
light and shadow on said surface in the  
presence of dry adsorbed chlorine gas for  
reproducing said image in tangible form on  
80 said surface, then fixing said image on said  
surface by subjecting the same to an electric  
current while said surface is immersed in a  
bath compounded as follows, distilled water,  
85 1500 cubic centimeters, nickel ammonium  
sulphate, 5 grams, sodium chromate, 5 grams,  
and ammonium bisulphate, 5 grams, then  
covering said surface with a transparent  
90 lacquer.

8. The herein described process of repro-  
ducing images on metallic surfaces, comprising providing a metal of a group consisting  
95 of iron, steel Monel metal, brass and copper  
with a highly polished surface, then subject-  
ing a film with images to light and register-  
ing said image in light and shadow on said  
surface in the presence of dry adsorbed  
100 chlorine gas for reproducing said image in  
tangible form on said surface, then fixing  
said image on said surface by subjecting the  
same to an electric current while said surface  
is immersed in a bath compounded as fol-  
105 lows, distilled water, 1500 cubic centimeters,  
nickel ammonium sulphate, 5 grams, sodium  
chromate, 5 grams, and ammonium bisul-  
phate, 5 grams, then covering said surface with a  
110 transparent lacquer.

9. The herein described process of repro-  
ducing images on metallic surfaces, comprising  
115 the subjecting of a film to dry chlorine gas  
for a period of an hour or more, then placing  
the same on a highly polished iron surface,  
then placing a negative with images thereon  
over said chlorine treated film and subjecting  
120 the same to light.

10. The herein described process of repro-  
ducing images on metallic surfaces, comprising  
125 the subjecting of a film to dry chlorine gas  
for a period of an hour or more, then placing  
the same on a highly polished Monel metal

surface, then placing a negative with images thereon over said chlorine treated film and subjecting the same to light.

11. The herein described process of reproducing images on metallic surfaces, comprising the subjecting of a film to dry chlorine gas for a period of an hour or more, then placing the same on a highly polished copper surface, then placing a negative with images thereon over said chlorine treated film and subjecting the same to light.

12. The herein described process of reproducing images on iron surfaces, comprising providing said iron with a highly polished surface, then placing a film with said image in contact with said surface and subjecting it to light in the presence of dry adsorbed chlorine gas for reproducing said image in tangible form on said surface.

13. The herein described process of reproducing images on Monel metal surfaces, comprising providing said Monel metal with a highly polished surface, then placing a film with said image in contact with said surface and subjecting it to light in the presence of dry adsorbed chlorine gas for reproducing said image in tangible form on said surface.

14. The herein described process of reproducing images on metallic surfaces, comprising the subjecting of a film to dry chlorine gas for a period of an hour or more, then placing the same on a highly polished iron surface, then placing a negative with images thereon over said chlorine treated film and subjecting the same to light, then placing said iron surface in a bath compounded as follows: distilled water 1500 cubic centimeters, nickel ammonium sulphate 5 grams, sodium chromate 5 grams, and ammonium bisulphate 5 grams, and while submerged in said bath subjecting said surface to a current of electricity, then washing the iron surface and drying the same, then covering said surface with a fine transparent lacquer.

15. The herein described process of reproducing images on metallic surfaces, comprising the subjecting of a film to dry chlorine gas for a period of an hour or more, then placing the same on a highly polished Monel metal surface, then placing a negative with images thereon over said chlorine treated film and subjecting the same to light, then placing said Monel metal surface in a bath compounded as follows, distilled water 1500 cubic centimeters, nickel ammonium sulphate 5 grams, sodium chromate 5 grams, and ammonium bisulphate 5 grams, and while submerged in said bath subjecting said surface to a current of electricity, then washing the Monel metal surface and drying the same, then covering said surface with a fine transparent lacquer.

16. The herein described process of reproducing images on metallic surfaces, comprising the subjecting of a film to dry chlorine

gas for a period of an hour or more, then placing the same on a highly polished copper surface, then placing a negative with images thereon over said chlorine treated film and subjecting the same to light, then placing said copper surface in a bath compounded as follows, distilled water 1500 cubic centimeters, nickel ammonium sulphate 5 grams, sodium chromate 5 grams, and ammonium bisulphate 5 grams, and while submerged in said bath subjecting said surface to a current of electricity, then washing the copper surface and drying the same, then covering said surface with a fine transparent lacquer.

17. The herein described process of reproducing images on metallic surfaces, comprising the subjecting of a film to dry chlorine gas for a period of an hour or more, then placing the same on a highly polished metallic surface of a material selected from a group consisting of any metal which is responsive to the action of chlorine gas when exposed to light, then placing a negative with images thereon over said chlorine treated film and subjecting the same to light.

18. The herein described process of reproducing images on metallic surfaces, comprising the subjecting of a film to dry chlorine gas for a period of an hour or more, then placing the same on a highly polished metallic surface of a material selected from a group consisting of any metal which is responsive to the action of chlorine gas when exposed to light, then placing a negative with images thereon over said chlorine treated film and subjecting the same to light, then placing said metallic surface in a bath compounded as follows, distilled water, 1500 cubic centimeters, nickel ammonium sulphate, 5 grams, sodium chromate, 5 grams, and ammonium bisulphate, 5 grams, and while submerged in said bath subjecting said surface to a current of electricity of 10 volts for one second, then washing the metallic surface and drying the same, then covering said surface with a fine, transparent lacquer.

19. The herein described process of reproducing images on metallic surfaces, comprising providing a metal of a material selected from a group consisting of any metal responsive to the action of chlorine gas when exposed to light, then subjecting a transparent member to dry chlorine gas for a period of an hour or more, then placing said transparent member against said surface, then placing a negative with an image in contact with said chlorine gas treated film and then subjecting the same to light, then electroplating said surface.

20. The herein described process of reproducing images on metallic surfaces, comprising providing a metal of a material selected from a group consisting of any metal responsive to the action of chlorine gas when exposed to light, then subjecting a transpar-

ent member to dry chlorine gas for a period of an hour or more, then placing said transparent member against said surface, then placing a negative with an image in contact with said chlorine gas treated film, then subjecting the same to light, then electroplating said surface, then covering said surface with a transparent lacquer.

21. The herein described process of reproducing images on metallic surfaces, comprising providing a metal of a material selected from a group consisting of any metal responsive to the action of chlorine gas when exposed to light, then subjecting a film with images to light and registering said image in light and shadow on said surface in the presence of dry absorbed chlorine gas for reproducing said image in tangible form on said surface, then fixing said image on said surface by subjecting the same to an electric current while said surface is immersed in a bath compounded as follows, distilled water, 1500 cubic centimeters, nickel ammonium sulphate, 5 grams, sodium chromate, 5 grams, and ammonium bisulphate, 5 grams.

In testimony whereof, I have hereunto set my hand at San Diego, California this 21st day of February 1929.

JOHN P. BROCKWAY.

30

35

40

45

50

55

60